

2. Sheets. Sheet 1.  
Paul & Wood,

Amalgamator.

No. 95,931.

Patented Oct. 19, 1869.

FIG  
1



FIG 2



WITNESS

Hate. M. Atkinson  
M. B. Dennis

INVENTORS

Almonin B. Paul.  
J. L. Wood  
By his Attorney  
J. H. Atkinson

Paul & Wood, 2. Streets. Street 2.

Amalgamator:

No. 95931.

Patented Oct. 19. 1869.

FIG. 3



FIG. 2: A



INVENTORS

WITNESS

State. M. Atkinson  
R. B. Blommy

Almarus B. Paul.  
I. L. Wood  
By his Attorney  
J. H. Atkinson

# United States Patent Office.

ALMARIN B. PAUL, OF SAN FRANCISCO, AND J. L. WOOD, OF INDEPENDENCE, CALIFORNIA.

Letters Patent No. 95,931, dated October 19, 1869.

## IMPROVED PROCESS FOR AMALGAMATING GOLD AND SILVER.

The Schedule referred to in these Letters Patent and making part of the same

*Know all men by these presents:*

That we, ALMARIN B. PAUL, of the city and county of San Francisco, California, and J. L. WOOD, of Independence, Inyo county, California, have made a new and useful invention for the Amalgamating of Gold and Silver, which is called "The Paul and Wood Electric Amalgamating-Process;" the following, taken together with the drawing, figures, and letters attached, being a full and exact description thereof.

The nature of our improvement consists in amalgamating the ores of the precious metals, in a perfectly pulverized and dry condition, by means of a simple and horizontal metallic barrel or cylinder, and the addition of mercury.

To enable others skilled in the art to understand and use our invention, and the process of amalgamation therewith, we will proceed to describe the same.

A, figs. 1 and 2, is a horizontal hollow metallic cylinder, suspended or supported on its hollow axles, by means of suitable bearings in the chamber of the furnace.

By means of the hollow axles, communication with the cylinder from the atmosphere is made.

On one of the axles is a pulley, for giving a rotary motion to the cylinder.

Below the cylinder is a space for a fire-hearth, or grate, and at any suitable part of the furnace a chimney or place may be constructed for carrying off the smoke or gas from any fire that may be made therein.

The cylinder is also provided with a proper opening, at any suitable place, for the introduction of materials thereto, and for withdrawing the same.

This opening is provided with a proper cover for closing it.

The inside of the cylinder is left smooth, as it may be left, by casting, or by wrought-iron materials.

The process of amalgamation with the above-described apparatus is as follows, viz:

The metalliferous ore, finely pulverized, is placed in the cylinder A, in such a quantity as to occupy less depth than one-half of its diameter. The opening is then closed. The cylinder is then set in slow motion, and a gentle fire applied in the grate, or on the hearth below it, for the purpose of completely but

slowly drying and ventilating the pulverized ore, the moisture escaping therefrom through the hollow axles B B.

When the drying-process is finished, the fire is allowed to go out, as it is no longer needed, the hollow axles stopped up, and the mercury in a large amount, greater than in ordinary processes, and according to the different natures of the ores to be treated, introduced into the cylinder, through the openings thereof, which is then closed.

The amalgamation now begins, and goes on by the slow revolution of the cylinder, and its contents, by which the mercury is thoroughly incorporated with the ore, the slight heat induced therein by the previous drying-process being sufficient to give a proper tenacity to the mercury, without vaporizing or volatilizing it, for its more perfect dissemination through the pulverized ore.

Figure 1, front view.

Figure 2, cylinder or barrel.

Figure 3, end view.

A, barrel.

B, axles.

C, opening.

D, fire-bed.

We do not claim the use of the hollow cylinder, for the purpose either of roasting, desulphurizing, vaporizing, or volatilizing; neither do we claim the hollow axles for the introduction and use of the vapors of mercury, for purposes of amalgamation; but

We do claim—

1. The combination of the simple horizontal rotating hollow or perforated-axed cylinder A, with a furnace, for the purpose of drying and ventilating materials to be amalgamated.

2. The process of drying and ventilating metalliferous ores, and amalgamating the same, substantially as set forth.

3. The amalgamating of pulverized ores in a dry condition, with mercury, in metallic or wooden barrels or cylinders, without the use of artificial heat.

ALMARIN B. PAUL.  
J. L. WOOD.

Witnesses:

CALVIN BROWN,  
FRANK E. BROWN.